

## UNITED STATES PATENT OFFICE

2,355,257

## MINERAL OIL COMPOSITION

Darwin E. Badertscher, Woodbury, N. J., assignor  
to Socony-Vacuum Oil Company, Incorporated,  
a corporation of New York

No Drawing. Application June 11, 1943,  
Serial No. 490,479

13 Claims. (Cl. 252—51)

This invention has to do with the stabilization of mineral oil fractions and more particularly has to do with the stabilization of such fractions by the incorporation therein of a small amount of a novel compound, or novel class of compounds, capable of inhibiting a viscous mineral oil against the deleterious effects of oxidation.

It is well known to those familiar with the art that the deleterious effects of oxidation upon a mineral oil fraction manifests itself in various ways depending upon the source of the oil, that is, the crude from which it is derived, the refining treatment to which the oil has been subjected and the particular conditions under which the oil is subjected to oxidation. For example, mineral oil fractions refined for use as lubricants have a tendency to oxidize under conditions of use with the formation of sludge or acidic oxidation products. Also, in the case of internal combustion engines, particularly those operating with high cylinder pressures, there is a decided tendency for the ordinary lubricating oil fractions to form carbonaceous deposits which cause the piston rings to become stuck in their slots and which fills the slots in the oil ring or rings, thus materially reducing the efficiency of the engine.

Among the numerous improving agents proposed for use in mineral oil fractions are various metal salts and metallo-organic compounds. While such metal compounds are generally effective in mineral oils, they are somewhat undesirable inasmuch as they are, generally, relatively insoluble in non-associated solvents such as mineral oils and the like. In contrast to these metal compounds are chelate metal salts which are much more soluble in non-associated solvents and less soluble in associated solvents than non-chelate metal salts. In short, the chelate metal salts are much more "organic" in nature in that they possess relatively low melting points and high vapor pressures in addition to increased solubility in non-associated solvents. Further distinctions between chelate metal salts and non-chelate metal salts may be obtained by referring to Sidgwick's "The Electronic Theory of Valence," Oxford University Press, 1927, chapter 14.

The oil improving agents contemplated herein, which effectively stabilize mineral oil fractions against the deleterious effects of oxidation, are the chelate metal salts of a salicylidene imine

which may be unsubstituted or substituted. These metal salts may be represented by the following general formula:



wherein R is selected from the group consisting of hydrogen and hydrocarbon radicals such as alkyl, alkaryl, and aralkyl; and radicals such as alkoxy, aroxy, halogen, nitro, nitroso and cyano; R' is selected from the group consisting of hydrogen and hydrocarbon radicals such as alkyl, aryl, alkaryl and aralkyl; and M represents the hydrogen equivalent of a metal.

All metals capable of forming chelate metal salts are contemplated as constituents of the metal salts described above. Illustrative of such metals are: sodium, copper, beryllium, magnesium, boron, aluminum, silicon, arsenic, antimony, chromium, iron, cobalt, nickel, palladium, platinum and iridium. Particularly preferred of such metal constituents are the metals nickel, copper and cobalt in the following forms: nickelous, cupric and cobaltous.

While the imino hydrogen (=N—H) may be present in the metal salts contemplated herein, it is preferred that the imino hydrogen be replaced by a hydrocarbon radical such, for example, as an alkyl or an aryl radical. Radicals representative of these classes are butyl, dodecyl and tolyl.

Although the metal salts of unsubstituted and N-substituted salicylidene imine are preferred herein, the metal salts of C-substituted salicylidene imine, which are those having groups substituted for nuclear hydrogen, are also effective mineral oil improving agents and consequently are contemplated herein. Typical of the C-substituents are alkyl, aralkyl and alkaryl groups.

The chelate metal salts of the type defined above may be prepared by the general method described in detail by Hunter and Marriott in the Journal of the Chemical Society (London)

1937, page 2000. Illustrative of the general method and of the chelate metal salts prepared thereby are the following examples.

**EXAMPLE I**  
*Nickelous salicylidene N-n-butyl imine*

A hot solution of 17.5 grams of salicylaldehyde in 20 cc. of 95% ethanol was added to a hot solution of 11 grams of mono-n-butyl amine in 20 cc. of 95% ethanol, the latter solution being constantly agitated. The reaction was strongly exothermic and caused the mixture to boil vigorously. A hot solution of 18 grams of nickelous acetate,  $\text{Ni}(\text{OAc})_2 \cdot 4\text{H}_2\text{O}$ , in 100 cc. of 50% aqueous ethanol was added to the aforesaid mixture, with constant agitation. About 44.5 grams of alcoholic potassium hydroxide containing 18.2% of 85% potassium hydroxide was then added. A dark green oil immediately formed and crystallized on cooling. The olive green crystals obtained by filtering the last mentioned mixture were washed on the filter with distilled water, then with 50 cc. of 95% ethanol in three portions and finally with 20 cc. of absolute ethanol. Crystallization from acetone yielded dark olive green crystals melting sharply at 139.5-140° C. (uncorrected). On analysis the following data was obtained.

| Analysis      | Found   | Cal'd. for<br>$\text{C}_{14}\text{H}_{18}\text{N}_2\text{O}_2\text{Ni}$ |
|---------------|---------|-------------------------------------------------------------------------|
|               | Percent | Percent                                                                 |
| Nickel.....   | 14.62   | 14.3                                                                    |
| Nitrogen..... | 6.46    | 6.83                                                                    |

**EXAMPLE II**

*Cupric salicylidene N-n-butyl imine*

To a hot solution of 8.2 grams of cupric acetate monohydrate and 6 grams of mono-n-butyl amine in 120 cc. of 50% aqueous ethanol was added, with shaking, a solution of 10 grams of salicylaldehyde in 10 cc. of 95% ethanol. After the mixture had cooled, the dark olive green crystals formed thereon were filtered, washed in the filter first with distilled water and then with absolute ethanol and were finally air dried. Analysis of these crystals showed the following:

| Analysis      | Found   | Cal'd. for<br>$\text{C}_{14}\text{H}_{18}\text{N}_2\text{O}_2\text{Cu}$ |
|---------------|---------|-------------------------------------------------------------------------|
|               | Percent | Percent                                                                 |
| Copper.....   | 15.28   | 15.4                                                                    |
| Nitrogen..... | 6.44    | 6.8                                                                     |

**EXAMPLE III**

*Cobaltous salicylidene N-n-butyl imine*

This material was prepared from 25 grams of salicylaldehyde, 15 grams of mono-n-butyl amine and 24.5 grams of cobaltous acetate tetrahydrate using a procedure similar to that described in Example I. The product was a crystalline, brick red solid which analyzed as follows:

| Analysis      | Found   | Cal'd. for<br>$\text{C}_{14}\text{H}_{18}\text{O}_2\text{N}_2\text{Co}$ |
|---------------|---------|-------------------------------------------------------------------------|
|               | Percent | Percent                                                                 |
| Nitrogen..... | 6.7     | 6.05                                                                    |
| Cobalt.....   | 14.3    | 16.87                                                                   |

**EXAMPLE IV**

*Cobaltous salicylidene N-n-dodecyl imine*

5 A hot solution of 25 grams (excess) of salicylaldehyde in 30 cc. of absolute ethanol was added to a hot solution of 37 grams of mono-n-dodecyl amine in 70 cc. of 95% ethanol, the mixture being agitated throughout the addition. The reaction was exothermic causing the mixture to boil vigorously. To the resulting mixture was added a solution of 25 grams of cobaltous acetate tetrahydrate in a mixture of 50 cc. of water and 60 cc. of 95% ethanol. The light yellow imine solution immediately turned brown on addition of the cobalt salt. After heating on the hot plate at a temperature of about 60° C. for about ten minutes with shaking, 77-78 grams of 14% alcoholic potassium hydroxide was added. The mixture now became green due to the separation of a dark green liquid phase. Five hundred cc. of distilled water were added to the reaction mixture and the resulting mixture was extracted thoroughly with petroleum ether until the petroleum ether extracts were no longer colored. On evaporation of petroleum ether from the extracts, 57.5 grams of a dark green pasty residue were obtained. A small drop of this residue fused in a porcelain crucible with about 2 to 3 cc. of borax gave a brilliant blue coloration, indicating the presence of cobalt.

10 To demonstrate the effectiveness of the salts contemplated herein as oil improving agents, a blank oil and blends of typical improving agents of the type contemplated herein were subjected to an oxidation test in order to determine their relative susceptibility to oxidation. In this test a 300 gram sample of the blank oil or of the oil blend was heated at 350° F. while two liters of air per hour were blown over their respective surfaces and while stirring the samples at a constant rate with steel paddles. The oil used was a commercial, solvent-refined S. A. E. 30 motor oil. Samples were withdrawn at specified intervals (in days) and the volume per cent of sludge was determined in each case. The results are set forth below in Table 1.

20

Table 1

| Improving agent added to oil             | Per cent | Sludge volume, per cent |        |         |         |         |         |
|------------------------------------------|----------|-------------------------|--------|---------|---------|---------|---------|
|                                          |          | 7 days                  | 9 days | 10 days | 11 days | 12 days | 13 days |
| None                                     |          | 12                      | 25     |         |         |         |         |
| Nickelous salicylidene N-n-butyl imine   | 0.25     | 5                       | —      | 15      | —       | —       | —       |
| Cobaltous salicylidene N-n-butyl imine   | 0.25     | 0                       | 0      | —       | 3       | —       | 20      |
| Cobaltous salicylidene N-n-dodecyl imine | 1.0      | 0                       | 0      | —       | —       | 15      | —       |

30

40 In order to evaluate the relative stability of a motor oil and of blends of the same motor oil and typical improving agents of the type contemplated herein the blank oil and the blends were tested in a standard C. F. R. "knock test" engine. The test involved operating the engine first with the oil and then with the oil blend at an approximate speed of 1200 R. P. M. with the throttle set just below detonation using a compression ratio of 7:1 at a fixed jacket temperature of 400° F.

At the end of 28 hours, the following inspections were made:

1. The piston:

- Degree of ring sticking (0° being an entirely free ring and 360° a totally stuck ring)
- Per cent of filling of oil slots
- Deposits (grams)

2. Used oil:

- Kinematic viscosity (K. V.) at 210° F.
- Neutralization number (N. N.)

The results obtained are listed below in Table 2 where oil A is a motor oil blank, oil B is the same oil containing 0.5 per cent of nickelous salicylidene N-n-butyl imine and oil C is the same oil containing 1 per cent of nickelous salicylidene N-n-dodecyl imine.

Table 2

| Oil   | Rings, degrees stuck |     |     |     |     | Slots, per cent filled | Total deposits, grams | Used oil        |       |
|-------|----------------------|-----|-----|-----|-----|------------------------|-----------------------|-----------------|-------|
|       | 1                    | 2   | 3   | 4   | 5   |                        |                       | K. V. @ 210° F. | N. N. |
| Oil A | 60                   | 180 | 360 | 360 | 360 | 00                     | 80                    | 75              | 14.3  |
| Oil B | 0                    | 0   | 0   | 0   | 0   | 0                      | 0                     | 0               | 28.77 |
| Oil A | 360                  | 360 | 360 | 360 | 360 | 00                     | 80                    | 95              | 4.9   |
| Oil C | 0                    | 0   | 0   | 0   | 0   | 0                      | 0                     | 0               | 24.67 |
|       |                      |     |     |     |     |                        |                       |                 | 1.0   |
|       |                      |     |     |     |     |                        |                       |                 | 0.4   |
|       |                      |     |     |     |     |                        |                       |                 | 1.8   |
|       |                      |     |     |     |     |                        |                       |                 | 0.4   |

The amount of improving agents which may be used in the oil will vary more or less with the oil and with the conditions of use. While in general the desired improvement can be effected with amounts ranging from about 0.01 per cent to about 10 per cent, the preferred amounts will fall within the range of about 0.1 per cent to about 5 per cent depending on solubility.

It is to be understood that while we have described hereinabove preferred procedures for synthesizing improving agents of the type contemplated herein and have designated certain illustrative reactants and have also shown certain preferred mineral oil fractions which may be employed, the invention is not confined to the specific detailed procedural operations, reactants or oils so described but includes within its scope whatever changes fairly come within the spirit of the appended claims.

I claim:

- An improved mineral oil composition comprising a viscous mineral oil having in admixture therewith a minor proportion, sufficient to stabilize said mineral oil against the deleterious effects of oxidation, of a chelate metal salt of a salicylidene imine, said salt being represented by the formula



wherein R and R' are selected from the group consisting of hydrogen and a hydrocarbon radical and M is the hydrogen equivalent of a metal possessed of the capacity to form a chelate metal salt.

- An improved mineral oil composition comprising a viscous mineral oil having in admixture

therewith a minor proportion, from about 0.01 per cent to about 10 per cent, of a chelate metal salt of a salicylidene imine, said salt being represented by the formula



wherein R and R' are selected from the group consisting of hydrogen and a hydrocarbon radical and M is the hydrogen equivalent of a metal possessed of the capacity to form a chelate metal salt.

- An improved mineral oil composition comprising a viscous mineral oil having in admixture therewith a minor proportion, sufficient to stabilize said mineral oil against the deleterious effects of oxidation, of a chelate metal salt of a salicylidene imine, said salt being represented by the formula



wherein R and R' are selected from the group consisting of hydrogen and a hydrocarbon radical and M is the hydrogen equivalent of a metal possessed of the capacity to form a chelate metal salt and is selected from the group consisting of copper, cobalt and nickel.

- An improved mineral oil composition comprising a viscous mineral oil having in admixture therewith a minor proportion, sufficient to stabilize said mineral oil against the deleterious effects of oxidation, of a chelate metal salt of a salicylidene imine, said salt being represented by the formula



wherein R and R' are selected from the group consisting of hydrogen and a hydrocarbon radical and M is the hydrogen equivalent of a metal possessed of the capacity to form a chelate metal salt and is selected from the group consisting of copper (cupric), cobalt (cobaltous) and nickel (nickelous).

- An improved mineral oil composition comprising a viscous mineral oil having in admixture therewith a minor proportion, sufficient to stabilize said mineral oil against the deleterious effects of oxidation, of a chelate metal salt of salicylidene imine.

An improved mineral oil composition comprising a viscous mineral oil having in admixture therewith a minor proportion, sufficient to stabilize said mineral oil against the deleterious effects of oxidation, of a chelate metal salt of an N-substituted salicylidene imine.

- An improved mineral oil composition comprising a viscous mineral oil having in admixture therewith a minor proportion, sufficient to stabilize said mineral oil against the deleterious

- effects of oxidation, of a chelate metal salt of an N-aryl substituted salicylidene imine.
8. An improved mineral oil composition comprising a viscous mineral oil having in admixture therewith a minor proportion, sufficient to stabilize said mineral oil against the deleterious effects of oxidation, of a chelate metal salt of an N-alkyl substituted salicylidene imine.
9. An improved mineral oil composition comprising a viscous mineral oil having in admixture therewith a minor proportion, sufficient to stabilize said mineral oil against the deleterious effects of oxidation, of a chelate metal salt of a C-substituted salicylidene imine.
10. An improved mineral oil composition comprising a viscous mineral oil having in admixture therewith a minor proportion, sufficient to stabilize said mineral oil against the deleterious effects of oxidation, of a chelate metal salt of an N-substituted, C-substituted salicylidene imine.

11. An improved mineral oil composition comprising a viscous mineral oil having in admixture therewith a minor proportion, sufficient to stabilize said mineral oil against the deleterious effects of oxidation, of nickelous salicylidene N-n-butyl imine.

12. An improved mineral oil composition comprising a viscous mineral oil having in admixture therewith a minor proportion, sufficient to stabilize said mineral oil against the deleterious effects of oxidation, of cobaltous salicylidene N-n-dodecyl imine.

13. An improved mineral oil composition comprising a viscous mineral oil having in admixture therewith a minor proportion, sufficient to stabilize said mineral oil against the deleterious effects of oxidation, of cobaltous salicylidene N-n-butyl imine.

DARWIN E. BADERTSCHER.